

April 5, 1966

J. R. MURLEY

3,244,275

CRIMPED STAPLE FIBRES

Filed April 2, 1963



"DEAD" BALE HAVING REDUCED TENDENCY TO EXPAND AFTER THE STRAPS ARE CUT

Fig. 2



COMPRESSED, RANDOMLY ARRANGED, UNFUSED STAPLE FIBERS HAVING THREE DIMENSIONAL CRIMP PRODUCED BY THE BALING OPERATION



Fig. 3

INVENTOR  
JOHN R. MURLEY

Cushman, Darby & Cushman  
ATTORNEYS

# United States Patent Office

3,244,275  
Patented Apr. 5, 1966

1

3,244,275

## CRIMPED STAPLE FIBRES

John Reginald Murley, Harrogate, England, assignor to Imperial Chemical Industries Limited, London, England, a corporation of Great Britain

Filed Apr. 2, 1963, Ser. No. 269,892

12 Claims. (Cl. 206—83.5)

This invention relates to a process for making crimped staple fibres from synthetic fibre forming polymers, particularly those made from polyethylene terephthalate.

I have found unexpectedly that a 3 dimensional crimp and deformations in cross-section can be obtained in staple fibres made from synthetic fibre forming polymers by submitting a bulk quantity of randomly arranged fibres to mechanical compression for example between the platens of a baling press. Unidirectional compression of a bulk quantity of substantially randomly laid fibres has been found to give the desired result but it will be appreciated that compression in more than one direction simultaneously or in succession will give the desired result e.g. by compressing a bale first in one direction and then at right angles thereto, under suitable conditions. These conditions are quite critical but we have determined by research and experiment that they can be expressed very simply by reference to the ultimate density or true density of the fibres which are being so compressed.

I have found that the fibres after suitable compression in the bale, have a lesser tendency to recover with the result that retaining straps which are used for baling such fibres do not snap open with a great force when cut. Moreover and more importantly the fibres are deformed beyond the elastic limit and also a plastic deformation occurs in the cross-section of the fibre. Unexpectedly these deformations are of such a kind that contrary to expectations the textile processing of such fibres although it requires certain modifications is not only possible but in some cases facilitated. Uncrimped fibres of uniform cross-section cannot be processed on normal textile processing machinery including carding and spinning but when compressed according to my invention are found to have sufficient retentivity and cohesion with each other to allow lap formation and subsequently to make the spinning of such initially uncrimped fibres into yarns possible.

According to my invention, therefore I provide a process for making crimped staple fibres from synthetic fibre forming polymers, particularly those made from polyethylene terephthalate, comprising compressing a bale of substantially randomly arranged fibres to a density which is at least 50% of the density of a single fibre in the bale and maintaining this pressure for a time sufficient for deformation of the fibres in their longitudinal direction beyond the elastic limit and also of their cross-section involving a plastic deformation to take place so that the fibres when released from pressure upon examination show a 3 dimensional crimp and deformations and at least 20 deformations of the cross-section of the fibres per linear cm. of the fibre, without any fusing between individual fibres. The deformations are caused by compressing the fibres in contact with one another until a deformation beyond the elastic limit takes place at their contacting surfaces. In the case of staple fibres of about 1 to 10 inches in length and of deniers between 1 and 10, the length of the fibre is of course many times greater than the diameter and accordingly the deformations in a random array of fibres will be approximately 1 or 2 fibre diameters along the length. It will be appreciated that the deforming effect of one fibre from another with which it is in contact will depend on the angle between

2

the axis of the fibres at the point of contact and upon the inclination of the line which is perpendicular to the axis of both fibres and which passes through their mutual point of contact to the direction of external pressure application that is to say the line of travel of the platens of a baling press.

Generally I have found a compression of a multitude of randomly laid fibres in a bale of 50% to 80% of the density of the single fibre is required to achieve crimping and the deformation of the cross-section beyond the elastic limit. The timing of the compression has an effect on the recovery of the fibres. The bale should therefore be maintained in a highly compressed state at a density greater than that of the final bale for a period of at least  $\frac{1}{4}$ , preferably about  $\frac{1}{2}$ —1 minute, in order to appreciably reduce the tendency of the bale to recover from its compressed state. By this means it has been found possible to restrain a polyethylene terephthalate fibre bale of 46 lbs. per cu. ft. density after ultimate compression with the same number and size of steel straps as are necessary on a bale of the same weight but only of 11 lbs. per cu. ft. density. This lack of recovery has a further advantage inasmuch as the high density bale when released from its straps expands slowly and by only a small amount, compared with the immediate and extensive recovery of the low density bale which expands to about twice its bale length. I have found that the initial openness or lay of the fibres has a considerable effect on the pressures which are required to compress a bulk quantity to within the specified limit, in order to get the required amount of deformation.

If e.g. as occurs in practice, a large tow of crimped filaments is cut, the cut tufts of fibres tend to cohere due to the presence of finish composition on the fibres and due to the mechanical compression during any previous crimping. Such tufts have a density of about 4 lbs. per cu. ft. in the case of polyethylene terephthalate fibres. If such fibre tufts are separated after cutting by a fluid stream a much looser and desirably random distribution of fibres is obtained.

Compression is commercially conveniently carried out in a baling press capable of exerting the required compression of the fibres. The fibres may be crimped by known methods, or uncrimped fibres may be used. In the former case additional crimp in 3 dimensions is super-imposed on the existing sinusoidal or saw-tooth crimp; in the latter case a random 3 dimensional non-uniform crimp results provided of course the fibres are substantially randomly distributed during compression. Conveniently the fibres are compressed to the required high density already in the form of a bale but in this context it will be appreciated that by a bale we mean a bulk quantity of fibres exceeding at least 10 lbs. in weight, preferably 100—200 lbs. in weight.

The invention will be further understood from the following detailed description in conjunction with the drawings in which:

FIGURE 1 is a block diagram illustrating the process steps for producing crimped fibres in accordance with the principles of the present invention;

FIGURE 2 is a perspective view of a strapped bale of compressed fibres crimped by the process of the present invention; and

FIGURE 3 is a graph in which the density of the compressed fibres is plotted against applied pressure.

In my British Patent 777,113 an apparatus for baling resilient staple fibers is described using rams having a clearance of at least 1.5 mm. all around in the compression chamber. Bales of fibres can be compressed to a density of about 20 lbs. cu. ft. i.e. bales with a residual density of 11—15 lbs. per cu. ft. can be obtained with such

a baler. This is insufficient for the production of fibers of my invention having a three dimensional crimp and other deformations. However, by modifying the design of the baler, we can produce the required high density bales, e.g. by using the ram for feeding the fibers into the chamber, as the high compression ram, withdrawing the ram after that compression, until sufficient fiber has been compressed in a first direction until the prescribed density has been achieved and then continuing the operation as described, by compressing a number of layers using said ram for feeding the fibers, as part of one side of the compression chamber, before compressing the fibers in a direction at right angles with a second ram against a quantity of previously compressed fiber and forming the side of said chamber, thereby also achieving continuous operation.

It will be appreciated that other baling machines may be used which are capable of compressing fibers to the required density.

A bale formed according to the present invention is illustrated in FIGURE 2. It has been found, unexpectedly, that even these high compression bales when strapped are quite safe to handle and that the bale is quite "dead," that is to say, the straps do not snap open when cut, as happens with "live" bales which endanger the operator when the straps are cut. I have found that such "live" bales are obtained when compressing, for example, polyethylene terephthalate fibers to a density up to 40 lbs. per cu. ft.

Although my description and the examples refer particularly to polyethylene terephthalate fibers, I believe that my invention is applicable to other synthetic linear polymer fibers such as those made from copolymers based on terephthalic acid, polyamides, polyacrylonitrile, ethylene polymers particularly stereo-specific polypropylene, and other fiber forming vinyl type polymers and polyoxymethylene.

It should be appreciated that the bulk quantity of super compressed fibers should not be subjected to a heat setting treatment in this compressed form because of the poor heat transfer properties of the fibers and therefore a resultant uneven heat treatment.

As seen in FIGURE 3 when the density, in lb./cu. ft. of a bulk quantity of fibers is plotted against the applied pressure, in tons per sq. inch a curve is obtained which at first rises slowly but then turns steeply and continues in a substantially straight line with a clearly definable break before continuing in the steep rise in a line displaced substantially parallel with the line before the break, below. The break in the line is believed to coincide with the formation of the crimps and the deformations in the fibers, beyond their elastic limit.

The following examples illustrate but do not limit my invention.

#### Example 1

A 225,000 denier tow of 1½ denier polyethylene terephthalate filaments which have been drawn, crimped and heat set to give 12 to 20 sinusoidal crimps, substantially in one plane, were cut into cotton type staple lengths of 1½". The cut staple fibers were fed into a baling machine, in principle as described in British Patent 777,113, but in addition to the slight compression and instead of the light ram, a heavy ram was used, capable of compressing each pre-weighed lot of fibers to give a resulting bale density of 64.1 lbs. per cu. ft., when the ram formed the top of the compression chamber. At this stage, the second ram was brought into operation and the bale was compressed at right angles against a previously compressed bale, ejected and strapped as described in British Patent 777,113.

This bale which had been compressed to a density of 64.1 lbs./cu. ft. was inert, dead and safe to handle when the straps were cut or opened accidentally. The fibers had non-uniform three dimensional crimp and they could

be peeled off in "leather-like" layers and on working by hand quickly assumed a desirable bulk and soft handle. Satisfactory laps of fibers weighing 13½ ozs. per sq. yard were prepared.

Although it is not stated in the example, I have found that the distribution of finish which had been applied to the filaments is improved in my bales.

#### Example 2

- 10 A bale containing 1½ denier crimped and heat-set polyethylene terephthalate fibers 1½" long and prepared on a baling machine as described in principle in British Patent 777,113 of dimensions 20" x 18" x 42" with 4 straps passing across the 20" edge and encompassing the 15 bale longitudinally is placed in a vertical hydraulic baling press. The direction of travel of the platens is vertical and is parallel to the longest dimensions of the bale. The bale density is 11 lb./cu. ft. In the top and bottom platens of the press there are grooves to accommodate the straps. 20 The straps are tightened when the platens, originally a distance of 42" apart at the beginning of the compression stroke, are closed to 8". The force required to effect this compression is 320 tons. Those four sides of the bale which are not in contact with the platens are not 25 supported in any way. The bale is then compressed further by a force of 560 tons. This pressure is maintained for 30 seconds. The separation of the platens is now 7" the density about 66 lbs. per cu. ft. When the pressure is released the bale bulges between the straps. The approximate height of the bale is 14 inches. Surprisingly the bale expands in height but there is little change in the other dimensions. The bale density is 45 lbs./cu. ft. This bale is inert, dead and safe to handle when the straps are cut or opened accidentally. The fibers have a non- 35 uniform, three dimensional crimp and 60 deformations of cross-sections per inch. Only the usual amount of disturbance of the fibers as used with bales of a density of 11-20 lbs. per cu. ft. is required when transferring the 40 fibers to the aprons of an opening line, to restore the usual bulk. Satisfactory laps of fibers weighing 13½ oz. per sq. yard have been prepared.

#### Example 3

- 45 Three slabs of high density bales prepared as described 50 in Example 2 are pressed lightly together and strapped, the straps are removed before combining the three slabs. With each of the slabs weighing 120 lbs., a bale weighing 360 lbs. is obtained occupying a volume of only ¾ of a 120 lb. bale having a density of only 11 lbs. per cu. ft. This illustrates the saving which can be obtained in warehouse space and in shipping costs with my bales.

#### Example 4

- 55 A 120 lb. bale of randomly laid polyethylene terephthalate staple fibers 1½" long and of 1½ denier the fibers having an ultimate density of 86 lbs. per cu. ft. is compressed in a superdensity hydraulic baling press. The initial bale has an overall height of 40 inches and 36 inches across the straps and having a bulk density of 17.9% of the ultimate density. This bale is further compressed to an overall height of 15" and measuring 11" across the straps when released from pressure and having a bulk density of 52% of the ultimate density in its strapped condition. The bale is placed axially between the platens of the high density hydraulic press which are slotted to accommodate the straps, the load is raised to

40,000 tons

70 bale weight (lbs.)

the length of the bale in inches is then equal to  
bale weight (lbs.)

The density is 68% of the ultimate density. The bale is then strapped with four straps to give a strap tension of 50 lbs. per sq. inch on a power tool and the straps are sealed. The load on the platens of the press is then increased to 600 tons and held at this pressure for 1 minute until yielding of the fibres is complete. The density is 77% of the ultimate density of the fibres in this condition. The load is then released and the bale expands to an effective length in inches of bale weight divided by 10.5. This results in the density of the bale of 52% of the ultimate density.

*Example 5*

Three high density bales are combined in the same press and using the procedure as in the previous example, but the original straps are retained and the combination of bales is secured by a separate set of four straps.

*Example 6*

A bale of polypropylene is prepared using an apparatus as described in British Patent 777,113, a load of 350 tons is used to compress a bale so obtained, the bulk density of the polypropylene fibres was 38 lbs. per cu. ft., compared with 58 lbs. per cu. ft. for the polyethylene terephthalate fibres. Both these densities are equivalent to about 67% of the ultimate density of the fibre. The individual fibres when examined under the microscope were found to be similarly deformed as the polyethylene terephthalate fibres.

*Example 7*

A bale of polyethylene terephthalate staple fibres 1½ denier 1½" which had not been crimped but which were coated with a spin finish solution of polyethylene glycol monolaurate and a corrosion inhibitor were compressed into a high density bale as described in Example 4. On examination the fibres showed permanent deformations on the long and short fibre axes. The fibres were subjected to normal processing conditions at a temperature of 76° F. and 38% relative humidity resulting in a satisfactory ¼0 S cotton count yarn.

Two weights of opener lap were made, firstly, one of 13 oz. per yard and secondly one of 17 oz. per yard. The lighter lap licked at unrolling but the heavier lap did not. There was a deposit of loose fibres thrown out at the drawing stages. This example illustrates that the fibres can be processed on the cotton system without previous crimping.

What I claim is:

1. A process for imparting three-dimensional crimp to a mass of short lengths of fibres of synthetic fibre forming polymer comprising: compressing as a unit the whole mass of said fibres which are randomly arranged in contact with each other to a density which is at least as great as 50% of the density of a single fibre; and maintaining this compressive pressure for a period of time to cause deformation of a majority of the fibres in their longitudinal direction beyond their elastic limit and to cause plastic deformation in the cross section of a majority of the fibres thereby producing a three-dimensional crimp and at least 20 deformations of each fibre per linear centimeter thereof without any fusing between individual fibres.

2. A process according to claim 1 in which the deformations are caused by compressing the fibres in contact with one another until a deformation beyond the elastic limit takes place on their contacting surfaces and in which the fibres are 1 to 10 inches in length and of a denier between 1 and 10.

3. A process according to claim 1 in which a multitude of randomly laid fibres in said mass are compressed 50% to 80% of the density of a single fibre.

4. A process according to claim 1 in which said mass is maintained in a highly compressed state at a density greater than that of the final mass for a period of at least ¼ minute.

5. A process according to claim 1 in which the fibres are separated and opened after cutting by a fluid stream to obtain a looser desirably random distribution of fibres before compressing in a bale.

6. A process according to claim 1 in which the quantity of fibres being compressed exceeds 10 lbs. in weight.

7. A process according to claim 1 in which the fibres are synthetic linear polymer fibres of a fibre forming polymer selected from the group consisting of polyethylene terephthalate, copolymers based on terephthalic acid, polyamides, polyacrylonitrile ethylene polymers particularly stereo-specific polypropylene and fibre formed vinyl type polymers and polyoxymethylene polymer.

8. A process of imparting three-dimensional crimp to short lengths of fibres of synthetic fibre-forming polymer comprising: mechanically compressing into the form of a self-supporting bale at least a ten pound mass of said fibres which are randomly arranged in contact with each other, said compressing step being effected by a pressure such that, when compression pressure is plotted against the density of the mass of fibres there is obtained a curve which at first rises slowly but then turns steeply and continues in a substantially straight line with a clearly definable break before continuing in the steep rise in a line displaced substantially parallel with the line before the break; and maintaining this compressive pressure for a period of time to cause deformation of a majority of the fibres in their longitudinal direction beyond their elastic limit and to cause plastic deformation in the cross section of a majority of the fibres thereby producing a three-dimensional crimp and at least 20 deformations of each fibre per linear centimeter thereof without any fusing between individual fibres.

9. A strapped compressed bale of randomly arranged unfused staple fibres of polyethylene terephthalate, said fibres being of substantially uniform density and having a three-dimensional crimp and at least 20 deformations of each fibre per linear centimeter thereof, said bale having a mass of at least ten pounds and a density which is at least as great as 50% of the density of a single fibre, said bale having a reduced tendency to expand after having been compressed and thereby having a reduced tendency to cause baling straps to snap open when the straps are cut.

10. A compressed bale as in claim 9 wherein said fibres are between 1 and 10 inches in length and of deniers between 1 and 10, said deformations in the random array of fibres being about 1 to 2 fibre diameters along the lengths of said fibres and occurring at the contacting surfaces of said fibres.

11. A compressed bale as in claim 9 wherein said polyethylene terephthalate fibres are about one and one-half inches in length.

12. A compressed bale as in claim 11 wherein said polyethylene terephthalate fibres have a spin finish uniformly distributed thereon.

**References Cited by the Examiner**

**UNITED STATES PATENTS**

|           |        |         |            |
|-----------|--------|---------|------------|
| 2,311,174 | 2/1943 | Hitt    | 19—66      |
| 2,539,725 | 1/1951 | Caraher | 206—83.5   |
| 2,647,285 | 8/1953 | Pfau    | 28—72      |
| 2,707,806 | 5/1955 | Wilkie  |            |
| 2,780,838 | 2/1957 | Wilkie  | 206—83.5 X |

**FOREIGN PATENTS**

|         |        |          |
|---------|--------|----------|
| 338,269 | 6/1921 | Germany. |
|---------|--------|----------|

*TERON E. CONDON, Primary Examiner.*

*DONALD W. PARKER, Examiner.*

*L. K. RIMRODT, J. M. CASKIE,*

*Assistant Examiners.*